

## UNITED STATES PATENT OFFICE

2,507,714

## MAGNESIUM-BASE ALLOYS

Alfred H. Hesse, Worthington, Ohio, assignor, by  
mesne assignments, to Mathieson Chemical  
Corporation, a corporation of Virginia

No Drawing. Application September 14, 1945,  
Serial No. 616,160

1 Claim. (Cl. 75—168)

1

This invention relates to magnesium-base alloys and has for its object the provision of an improved magnesium-base alloy comprising lithium and zinc, together with one or more of the metals silver, cadmium and aluminum. More particularly, the invention provides an alloy comprising magnesium as the principal constituent, from around 1% to 13% of lithium, from 1% to 10% of zinc, and with one or more of the metals silver, cadmium or aluminum. The silver and cadmium may be present in amounts from 1% to 10% and parts of these metals may be replaced with aluminum. Aluminum may also be used without silver or cadmium in amounts from 0.5% to 6%. The alloys of the invention are characterized by low specific gravity, good ductility, high tensile strength and good cold-working properties. Certain of these alloys have excellent creep resistance and stability of tensile properties at room temperature. Some of them are susceptible to heat treatment.

The new alloys of the invention may be prepared by any of the usual melting processes with precautions to prevent an excessive sodium contamination. For example, the magnesium may be melted in an iron crucible under a suitable flux, and then zinc, silver, cadmium, or aluminum, is added, as required, followed by the addition of lithium. In order to avoid excessive oxidation of the lithium during the alloying process, it is advisable to use means for holding the lightweight lithium beneath the surface of the molten metal. An inverted perforated steel cup, such as a phosphorizing cup or an analogous device suitable for this purpose, may be used. Temperatures

of about 1300° to 1400° F. may be used for alloying operations. After thorough agitation to insure homogeneity, the melt is allowed to settle at temperatures sufficient to maintain it in a liquid state, after which it is decanted into molds. A suitable casting temperature is, for example, about 1320° F. The alloy may be cast directly into permanent molds without the necessity of providing a neutral or reducing atmosphere.

10 To insure the absence of harmful amounts of sodium or potassium, I prefer to prepare these alloys as described in my copending application, Serial No. 603,749, filed July 7, 1945. In accordance with that application, I prefer to use a flux made up of one part of lithium fluoride to three parts of lithium chloride. Use of such a flux serves to reduce the sodium and potassium content of the alloy. I may also treat the alloy by blowing the melt with a gas such as nitrogen or ammonia to accomplish a decrease in sodium or potassium.

15 In another aspect of the invention, the lithium chloride-lithium fluoride flux is thickened after the lithium addition by stirring a high melting-point oxide or compound into the flux. These materials, by thickening the flux, tend to cause a better flux-metal separation. Oxides found suitable for this purpose are molybdenum sesquioxide, vanadic acid, magnesium oxide, and boric anhydride. These oxides do not appear to enhance the properties of the alloys but do provide cleaner metals at lower melting losses. Illustrative examples of alloys of this invention are given 20 in the following table:

| No. | Percentages |      |    |    |    |     | Per cent<br>Elongation | Per cent<br>Reduction<br>in Area | Yield<br>Strength | Tensile<br>Strength |
|-----|-------------|------|----|----|----|-----|------------------------|----------------------------------|-------------------|---------------------|
|     | Mg          | Li   | Zn | Ag | Cd | Al  |                        |                                  |                   |                     |
| 1   | 81.9        | 10.1 | 4  | 4  | —  | —   | 11.6                   | 25.6                             | 41,200            | 45,100              |
| 2   | 81.9        | 10.1 | 4  | —  | 4  | —   | 18.0                   | 32.7                             | 40,900            | 44,100              |
| 3   | 84.8        | 6.4  | 4  | 1  | —  | 4   | 8.5                    | 11.7                             | 31,900            | 42,100              |
| 4   | 81.0        | 10.0 | 4  | 1  | —  | 4   | 24.3                   | 41.9                             | 33,200            | 37,400              |
| 5   | 78.3        | 9.7  | 6  | 6  | —  | —   | 9.2                    | 16.3                             | 39,200            | 51,500              |
| 6   | 73.0        | 12.0 | 5  | 5  | 5  | —   | 2.0                    | 3.3                              | 48,300            | 49,900              |
| 7   | 83.0        | 9.0  | 2  | —  | —  | 1   | 26.7                   | 57.0                             | 31,300            | 35,800              |
| 8   | 81.88       | 7.12 | 7  | —  | —  | 4   | 8.5                    | 10.4                             | 31,300            | 41,500              |
| 9   | 79.12       | 6.88 | 10 | —  | —  | 4   | 5.5                    | 7.0                              | 32,900            | 41,600              |
| 10  | 84.64       | 7.36 | 7  | —  | —  | 1   | 10.0                   | 11.1                             | 30,100            | 41,500              |
| 11  | 81.88       | 7.12 | 10 | —  | —  | 1   | 16.7                   | 20.0                             | 28,600            | 38,100              |
| 12  | 88.84       | 9.16 | 2  | —  | —  | 0.5 | 30.5                   | 63.0                             | 28,800            | 33,200              |
| 13  | 88.3        | 3.7  | 2  | —  | —  | 4   | 13.7                   | 14.6                             | 33,300            | 47,400              |
| 14  | 90.2        | 3.8  | 2  | —  | —  | 4   | 16.7                   | 23.8                             | 27,500            | 42,600              |
| 15  | 86.4        | 3.6  | 4  | —  | —  | 6   | 5.5                    | 8.2                              | 31,100            | 44,000              |
| 16  | 86.4        | 3.6  | 2  | —  | —  | 8   | 3.0                    | 3.2                              | 32,500            | 36,900              |
| 17  | 84.5        | 3.5  | 4  | —  | —  | 8   | 3.0                    | 4.7                              | 35,800            | 45,100              |
| 18  | 84.5        | 3.5  | 4  | —  | —  | 8   | 2.7                    | 4.0                              | 34,400            | 44,600              |

The above alloys had specific gravities varying from around 1.55 to 1.57.

The tensile properties were measured on  $\frac{3}{16}$ " rod, extruded from the castings.

Alloys Nos. 5 and 6 of the table show remarkable stability of physical properties at room temperature. Their creep properties are comparable to the best commercially available aluminum-base alloys.

Both of these alloys are susceptible to heat treatment. For example, the extruded hardness of No. 5, about 93 Rockwell "E," is lowered to 88 when quenched from 500° F. Following the quench, the hardness may then be increased to about 98 Rockwell "E" after a 200° F. aging treatment. Alloy No. 6 shows a hardness on extrusion of about 90 Rockwell "E." This is lowered to 77 by heating to from 500° to 700° F. and quenching. A sixteen hour heat treatment at 150° F. restores the hardness to approximately 96 Rockwell "E." Thus, these alloys should lend themselves readily to cold-forming in the soft or quenched condition, and when formed may be converted to a strong structural material by the low-temperature heat treatment.

In describing and in claiming the various percentages of metals used in the alloys, it is understood that they include the ordinary impurities found in the commercial metals. While lithium, as ordinarily produced, contains objectionable amounts of sodium, the sodium may be substantially eliminated by the methods of refining herein described.

## I claim:

A magnesium-base alloy comprising from 1% to 13% of lithium, from 1% to 10% of zinc, from 1% to 10% of at least one metal of the group consisting of silver and cadmium, from 0.5% to 6% of aluminum and the balance magnesium.

ALFRED H. HESSE.

## REFERENCES CITED

10 The following references are of record in the file of this patent:

## UNITED STATES PATENTS

| Number    | Name          | Date           |
|-----------|---------------|----------------|
| 2,226,550 | Burkhardt     | Dec. 31, 1940  |
| 2,261,905 | Nelson et al. | Nov. 4, 1941   |
| 2,305,825 | Burkhardt     | Dec. 22, 1942  |
| 2,317,980 | Dean          | May 4, 1943    |
| 2,385,685 | Busk          | Sept. 25, 1945 |

## FOREIGN PATENTS

| Number  | Country       | Date          |
|---------|---------------|---------------|
| 524,511 | Great Britain | July 30, 1940 |
| 361,086 | Germany       | Oct. 10, 1922 |
| 509,024 | Germany       | Oct. 6, 1930  |

## OTHER REFERENCES

A. P. C. application of Burkhardt, Serial No. 303,611, pub. May 4, 1943.

30 Henry et al., "Lithium-Magnesium Equilibrium Diagram," Trans. Amer. Inst. Mining and Metallurgical Engrs., 1934, vol. III, pp. 319-332.